

## UNITED STATES PATENT OFFICE

2,628,716

## FLOTATION PROCESS

William H. Hill, Mount Lebanon, Pa., assignor to  
Koppers Company, Inc., Pittsburgh, Pa., a cor-  
poration of Delaware

No Drawing. Application March 15, 1946,  
Serial No. 654,817

10 Claims. (Cl. 209—166)

1

This invention relates to froth flotation processes and more particularly is directed to froth flotation of sulphide minerals, and still more particularly to selective froth flotation of sulphide minerals such as zinc and copper sulphides.

This invention has for its principle objects to provide new reagents for carrying out froth flotation processes, to provide new and effective collectors for sulphide minerals; to provide new collectors capable of selectively floating sulphide minerals such as copper and zinc sulphide from pyrite or pyrrhotite; to effect economies through higher recoveries, higher strength concentrates, simplified operation and/or reduced operating time; to obtain advantages as will be pointed out; and to avoid the disadvantages of the prior art. Further objects will appear as the description proceeds.

These objects are accomplished in the present invention by carrying out froth flotation in the presence of a suitable thiopyrimidine. I have found that certain thiopyrimidines are effective collecting agents in the froth flotation of minerals, particularly sulphide minerals, and, because of their relative inability to float iron sulphides are particularly valuable in selective flotation of sulphide minerals containing pyrite or pyrrhotite. By means of the collectors of the invention, I am able to float a wide variety of minerals and in many instances, as, for example, with sulphite copper-iron ores and sulphide lead-zinc-iron ores to obtain improved concentrates and improved recovery along with greater flexibility of operation and shorter flotation periods.

Thiopyrimidines which are effective according to this invention, are compounds characterized by a 2-mercapto-1,3-diazine structure as represented by the following formula:



in which the R's are the same radical selected from the class consisting of methyl and ethyl radicals, such as may be obtained among other ways, by the condensation of ammonium thiocyanate with acetone or methyl ethyl ketone, or the corresponding alpha, beta unsaturated ketones resulting from the aldol condensation of acetone or methyl ethyl ketone. The products are well defined compounds being crystal-

2

line solids of low water solubility even in the form of their alkali metal salts.

These compounds may exist in one or more of the following tautomeric forms:



which accounts for the various names which have been applied to these in the prior art. The product obtained from mesityl oxide and ammonium thiocyanate, for example, is variously shown or designated as 2-mercapto-4,4,6-trimethyl-3,4-dihydropyrimidine or 2-mercapto-4,6,6-trimethyl-1,6-dihydropyrimidine (structure I); 2-thio-4,4,6-trimethyl-1,2,3,4-tetrahydropyrimidine or 2-thio-4,6,6-trimethyl-6,1,2,3-tetrahydropyrimidine (structure II); or 2-mercapto-4,4,6-trimethyl- or 2-mercapto-4,6,6-trimethyl dihydropyrimidine or 2-mercapto-4,4,6-trimethyl  $\Delta^{2,5}$  metadiazine (structure III) depending on the tautomeric form and whether the ring is numbered clockwise or counterclockwise. In the enol form the mercapto hydrogen may be replaced by inorganic radicals forming salts. Suitable methods for their preparation are disclosed in U. S.

15 Patents 2,131,790; 2,181,217; 2,234,848; and 2,244,547.

20 The compound 2-mercapto-4,4,6-trimethyl-3,4-dihydropyrimidine results also when acetone or diacetone is used instead of mesityl oxide. Thus 25 the same type of compound is obtained from ketones which by self condensation (aldol condensation) or by dehydration are capable of forming alpha, beta, unsaturated ketones.

30 Methyl ethyl ketone or its self condensation product, 5-methyl-4-penten-3-one, similarly condenses with ammonium thiocyanate to give 2-mercapto-4,6-diethyl-4-methyl-dihydropyrimidine. In the above formula this compound is represented when R is the ethyl radical. If the 35 ring is numbered counterclockwise, the name is 2-mercapto-4,6-diethyl-6-methyl-dihydropyrimidine as disclosed in U. S. Patent 2,356,710.

35 In carrying out flotation processes in accordance with the invention the thiopyrimidines as 40 described above are utilized to condition the mineral in essentially the same manner as standard collecting agents such as xanthates, dithiophosphates and substituted thioureas. They may be 45 incorporated in the mineral pulp in any suitable manner as, for example, in the liberation, clas-

50 55

sification or conditioning operations along with such other reagents as frothers, depressants, conditioners, other collectors, etc., as are commonly used or as may be desired, and the treated pulp subjected to froth flotation according to any suitable procedure.

The effectiveness of the compounds of the invention depends upon the nature of the ore, the amount used, the pH, the time and like factors. In short their efficiency depends upon the usual variables which affect the efficiency of collectors in froth flotation. In general, however, they are less susceptible to variation in pH and more effective in depressing pyrite and pyrrhotite and, in particular cases, float less insolubles and give lower tailings, higher concentrates and better over-all yields than collectors commonly used. Another advantage of the compounds of this invention is the fact that lime can be used to give the desired pH even in cases where other flotation agents now employed require the more costly soda ash as an alkalinizing agent. Thus while the collectors of this invention are generally useful in collecting a wide variety of minerals, particularly sulphide minerals, they are more particularly useful in effecting selective flotation of certain sulphide minerals such as copper and zinc ores containing relatively large quantities of

mesh, 46.2% minus 200 mesh with 6 lbs. of lime and 0.2 lb. of 2-mercaptop-4,4,6-trimethyl-3,4-dihydropyrimidine (obtained by the condensation of mesityl oxide with ammonium thiocyanate) per ton or ore. The ground ore was conditioned for 20 minutes and then subjected to a 10 minute flotation at 25% solids to which 0.1 lb. per ton pine oil was added one half at the start and the other half at five minutes. Two rougher concentrates were produced; the first taken for the first two minutes of the rougher float and the second for the last eight minutes. The results are tabulated below in Table I.

B. Procedure A was repeated except that 2-mercaptop-4,4,6-trimethyl-3,4-dihydropyrimidine was increased to 0.3 pound per ton of ore.

C. The ore was ground as in procedure A with 12 lbs. of lime per ton, conditioned for twenty minutes with 2 lbs. of sodium sulphite per ton and subjected to a ten minute flotation period at 25% solids to which 0.025 lb. Minerec B (Minerec B is a trade name for collectors obtained by dissolving a xanthate, probably potassium butyl xanthate, in ethyl chloro carbonate), 0.1 lb. of pine oil and 0.1 lb. potassium ethyl xanthate per ton were added. Two rougher concentrates were taken as in procedure A; the results are tabulated below in Table I.

Table I.—Flotation of copper sulfide according to the invention (A and B) as compared with the prior art (C)

| Procedure | Weight Percent Ro. Conc. |      | Percent Cu. Ro. Conc. |      | Percent Insoluble Ro. Conc. 1 | Percent Cu. Ro. Tails | Percent Cu. Recovery Ro. Conc. |     |
|-----------|--------------------------|------|-----------------------|------|-------------------------------|-----------------------|--------------------------------|-----|
|           | 1                        | 2    | 1                     | 2    |                               |                       | 1                              | 2   |
| A.....    | 24.9                     | 5.7  | 23.29                 | 4.73 | -----                         | 0.32                  | 92.2                           | 4.3 |
| B.....    | 23.1                     | 8.6  | 24.9                  | 4.53 | -----                         | 0.23                  | 91.3                           | 6.2 |
| C.....    | 23.4                     | 14.9 | 24.73                 | 2.56 | -----                         | 0.22                  | 91.8                           | 6.0 |

Ro. Conc.=Rougher Concentrate.

Ro. Tails=Rougher Tails.

pyrite. Thus through the collectors of the invention it is possible to produce a high grade copper concentrate essentially free of pyrite with relatively low insolubles from low grade sulphide copper-iron ores and to provide high grade zinc concentrates from sulphide zinc-iron ores with unusually high recoveries of zinc. Such terms as copper-iron ores and zinc-iron ores are intended to include virgin ores, concentrates, tailings and like products which contain the named metals with or without other values in admixture with gangue.

The amount required varies according to the particular ore and according to the effectiveness of the particular compound used but is of the same order of magnitude as the required amounts of like agents of the prior art. Suitable results have been obtained within the limits of 0.0025 to 0.025% by weight of the mineral (0.05 to 0.5 lb. per ton) but greater or lesser quantities may be used. For any particular compound and any particular mineral those skilled in the art, having in mind these principles will readily be able in view of the data given below to determine suitable amounts.

The invention may be more fully understood by reference to the following examples in which the parts are by weight unless otherwise specified.

#### EXAMPLE I

A. An Arizona sulfide copper-iron ore containing about 6% copper was ground to 4.0% plus 65

45 mesh, 46.2% minus 200 mesh with 6 lbs. of lime and 0.2 lb. of 2-mercaptop-4,4,6-trimethyl-3,4-dihydropyrimidine (obtained by the condensation of mesityl oxide with ammonium thiocyanate) per ton or ore. The ground ore was conditioned for 20 minutes and then subjected to a 10 minute flotation at 25% solids to which 0.1 lb. per ton pine oil was added one half at the start and the other half at five minutes. Two rougher concentrates were produced; the first taken for the first two minutes of the rougher float and the second for the last eight minutes. The results are tabulated below in Table I.

50

55

56

57

58

59

60

61

62

63

64

65

66

67

68

69

70

71

72

73

74

75

76

77

78

79

80

81

82

83

84

85

86

87

88

89

90

91

92

93

94

95

96

97

98

99

100

101

102

103

104

105

106

107

108

109

110

111

112

113

114

115

116

117

118

119

120

121

122

123

124

125

126

127

128

129

130

131

132

133

134

135

136

137

138

139

140

141

142

143

144

145

146

147

148

149

150

151

152

153

154

155

156

157

158

159

160

161

162

163

164

165

166

167

168

169

170

171

172

173

174

175

176

177

178

179

180

181

182

183

184

185

186

187

188

189

190

191

192

193

194

195

196

197

198

199

200

201

202

203

204

205

206

207

208

209

210

211

212

213

214

215

216

217

218

219

220

221

222

223

224

225

226

227

228

229

230

231

232

233

234

235

236

237

238

239

240

241

242

243

244

245

246

247

248

249

250

251

252

253

254

255

256

257

258

259

260

261

262

263

264

265

266

267

268

269

270

271

272

273

274

275

276

277

278

279

280

281

282

283

284

285

286

287

288

289

290

291

292

293

294

295

296

297

298

299

300

301

302

303

304

305

306

307

308

309

310

311

312

313

314

315

316

317

318

319

320

321

322

323

324

325

326

327

328

329

330

331

332

333

334

335

336

337

338

339

340

341

342

343

344

345

346

347

348

349

350

351

352

353

354

355

356

357

358

359

360

361

362

363

364

365

366

367

368

369

370

371

372

373

374

375

376

377

378

379

380

381

382

383

384

385

386

387

388

389

390

391

392

393

394

395

396

397

398

399

400

401

402

403

404

405

406

407

408

409

410

411

412

413

414

415

416

417

418

419

420

421

422

423

424

425

426

427

428

429

430

431

432

433

434

435

436

437

438

439

440

441

442

443

444

445

446

447

448

449

450

451

452

453

454

455

456

457

458

459

460

461

462

463

464

465

466

467

468

469

470

471

472

473

474

475

476

477

478

479

480

481

482

483

484

485

486

487

488

489

490

491

492

493

494

495

496

497

498

499

500

501

502

503

504

505

506

507

508

509

510

511

512

513

514

515

516

517

518

519

520

521

522

523

524

525

526

527

528

529

530

531

532

533

534

535

536

537

538

539

540

541

542

543

544

545

546

547

548

549

550

551

552

553

554

555

556

557

558

559

560

561

562

563

564

565

566

567

568

569

570

571

572

573

574

575

576

577

578

579

580

581

582

583

584

585

586

587

588

589

590

591

592

593

594

595

596

597

598

599

600

601

602

603

604

605

606

607

608

609

610

611

612

613

614

615

616

617

618

619

620

621

622

623

624

625

626

627

628

629

630

631

632

633

634

635

636

637

638

639

640

641

642

643

644

645

646

647

648

649

650

651

652

653

654

655

656

657

658

659

660

661

662

663

664

665

666

667

668

669

670

671

672

673

674

675

676

677

678

679

680

681

682

683

684

685

686

687

688

689

690

691

692

693

694

695

696

697

698

699

700

701

702

703

704

705

706

707

708

709

710

711

712

713

714

715

716

717

718

719

720

721

722

723

724

725

726

727

728

729

730

731

732

733

734

735

736

737

738

739

740

741

742

743

744

745

746

747

748

749

750

751

752

753

754

755

756

757

758

759

760

761

762

763

764

765

766

767

768

769

770

771

772

773

774

775

776

777

778

779

780

781

782

783

784

785

786

787

788

789

790

791

792

793

794

795

796

797

798

799

800

801

802

803

804

805

806

807

808

809

810

811

812

813

814

815

816

817

818

819

820

821

822

823

824

825

826

827

828

829

830

831

832

833

834

835

836

837

838

839

840

841

842

843

844

845

846

847

848

849

850

851

852

853

854

855

856

857

858

859

860

861

862

863

864

865

866

867

868

869

870

871

872

873

874

875

876

877

878

879

880

881

882

883

884

885

886

887

888

889

890

891

892

893

894

895

896

897

898

899

900

901

902

903

904

905

906

907

908

909

910

911

912

913

914

915

916

917

918

919

920

921

922

923

924

925

926

927

928

929

930

931

932

933

934

935

936

937

938

939

940

941

942

943

944

945

946

947

948

949

950

951

952

953

954

955

956

957

958

959

960

961

962

963

964

965

966

967

968

969

970

971

972

973

974

975

976

977

978

979

980

981

982

983

984

985

986

987

988

989

990

991

992

993

994

995

996

997

998

999

1000

addition of 0.05 lb. B23 alcohols and pine oil, 0.05 lb. potassium ethyl xanthate, 2.0 lbs. of lime and 0.5 lb. of copper sulfate per ton and subjected to a 10 minute flotation to give zinc rougher concentrate and tails. The results are given in Table II.

Table II.—Flotation of zinc sulfide according to the prior art

| Product       | Percent Wt. | Percent Composition |       |      | Percent Distribution |      |      |
|---------------|-------------|---------------------|-------|------|----------------------|------|------|
|               |             | Pb                  | Zn    | Fe   | Pb                   | Zn   | Fe   |
| Pb. Ro. Cone  | 19.1        | 70.2                | 3.42  | 2.4  | 96.2                 | 7.1  | 8.7  |
| Pb. Ro. Tails | 80.9        | 0.65                | 10.50 | 5.94 | 3.8                  | 92.9 | 91.3 |
| Heads         | 100         | 13.93               | 9.16  | 5.27 | 100                  | 100  | 100  |
| Zn. Ro. Conc. | 18.9        | 1.8                 | 43.48 | 2.5  | 2.4                  | 89.7 | 8.9  |
| Zn. Ro. Tails | 62.0        | 0.3                 | 0.47  | 7.0  | 1.4                  | 3.2  | 82.4 |
| Pb. Ro. Tails | 80.9        | 0.65                | 10.50 | 5.94 | 3.8                  | 92.9 | 91.3 |

B. The standard procedure was repeated substituting 0.2 lb./ton of 2-mercaptop-4,4,6-trimethyl-3,4-dihydropyrimidine for the 0.05 lb./ton of potassium ethyl xanthate in the zinc circuit. The results are given in Table III.

Table III.—Flotation of the sulfide according to the invention

| Product       | Percent Wt. | Percent Composition |      | Percent Distribution |       |
|---------------|-------------|---------------------|------|----------------------|-------|
|               |             | Zinc                | Fe   | Zn                   | Fe    |
| Pb. Ro. Cone  | 19.0        | 2.8                 | 1.8  | 5.9                  | 6.5   |
| Pb. Ro. Tails | 81.0        | 10.5                | 6.00 | 94.1                 | 93.5  |
| Heads         | 100.0       | 9.05                | 5.21 | 100.0                | 100.0 |
| Zn. Ro. Cone  | 16.0        | 52.42               | 2.2  | 92.7                 | 6.7   |
| Zn. Ro. Conc. | 65.0        | 0.20                | 6.95 | 1.4                  | 86.8  |
| Pb. Ro. Tails | 81.0        | 10.5                | 6.00 | 94.1                 | 93.5  |

From the data of Tables II and III it may be seen that process of the invention produced a zinc tail assaying less than half that obtained with xanthate and that the grade of concentrate was about 10% better.

The above procedures were carried out with fine ore because coarse zinc is generally difficult to float selectively. When the procedures were repeated with coarse ore, about 62% minus 200 mesh, the zinc tails in the standard increased from 0.47%, Table II, to 0.98%; whereas with 2-mercaptop-4,4,6-trimethyl-3,4-dihydropyrimidine the zinc tails increased only to 0.3%.

The collectors of the invention have also been found unusually effective in the treatment of marmatite ores, natural zinc-sulfide ores containing large amounts of pyrite. The collectors of the invention are unusually effective in floatating the zinc sulphides in these ores from the pyrite gangue. For example, marmatite zinc-iron ore assaying 0.04% lead and 5.42% zinc was subjected to froth flotation using 2-mercaptop-4,4,6-trimethyl-3,4-dihydropyrimidine in comparison with sodium isopropyl xanthate which is commonly used as a collector for this ore. In all tests a brittle froth was obtained with the xanthate making the froth removal from both rougher and cleaner cells difficult, whereas with the collector of the invention satisfactory frothing conditions were obtained throughout. The collector of the invention proved more selective in that considerably less circulating load was involved than obtained with the xanthate. The process of the invention also produced a higher grade cleaner concentrate assaying 46% zinc as compared with 43% for the xanthate. .2 lb. per ton or less of the collector of the invention

proved effective whereas .3 lb. per ton of the xanthate was required. The same collector of the invention was also found effective in floatating zinc sulphide in a marmatite zinc ore assaying 15.4% zinc, 0.4% lead and 30.4% iron. With the prior art collectors such as Aerofloat 25, soda

ash is required as the alkaline reagent. By using the collector of the invention it was found possible to obtain effective floatation with this ore using lime as the alkaline reagent, moreover the collector of the invention proved more potent and more selective in the lime circuit than the Aerofloat 25 in the soda ash.

The foregoing examples serve to illustrate typical embodiments of the invention and to point out some of the advantages of the invention with respect to the prior art practices. It is to be understood, however, that the invention is not limited to these particular embodiments or to any of the details thereof but that the invention may be variously embodied within the scope of the invention as outlined above and as set forth in the appended claims.

I claim:

1. In a process for froth floatation the steps of preparing a mineral pulp of a sulfidic ore, incorporating therein a thiopyrimidine having the following structure:



in which the R's are the same radical selected from the class consisting of methyl and ethyl radicals and subjecting the pulp to froth floatation.

2. In a process for froth floatation the steps of preparing a mineral pulp of a sulfidic ore, incorporating therein 2-mercaptop-4,4,6-trimethyl-3,4-dihydropyrimidine and subjecting the pulp to froth floatation.

3. In a process for froth floatation the steps of preparing a mineral pulp of a sulfide ore contaminated with pyrite incorporating therein a thiopyrimidine having the following structure:



in which the R's are the same radical selected from a class consisting of methyl and ethyl radicals and subjecting the pulp to froth floatation.

4. In a process for froth floatation the steps of preparing a mineral pulp of a sulphide ore contaminated with pyrite incorporating therein 2

mercapto - 4,4,6-trimethyl-3,4-dihydropyrimidine and subjecting the pulp to froth flotation.

5. The method of claim 4 in which the mineral is selected from the class consisting of sulphide copper-iron ores and sulphide zinc-iron ores.

6. In a method for selectively floating copper sulphide in a sulphide copper-iron ore the steps of preparing a mineral pulp of the ore, incorporating therein 2 mercapto-4,4,6-trimethyl-3,4-dihydropyrimidine and subjecting the pulp to 10 froth flotation.

7. In a method for separating lead, zinc and iron sulphides in sulphide lead-zinc-iron ores by means of froth flotation comprising the steps of selectively floating lead sulphide leaving a lead tails containing the bulk of the zinc and iron sulphides, and selectively floating zinc sulphide by subjecting said lead tails to froth flotation, the improvement which comprises effecting said froth flotation of said lead tails in the presence of a 15 thiopyrimidine of the formula:



in which the R's are the same radical selected from a class consisting of methyl and ethyl radicals. 30

8. In a method for separating lead, zinc and iron sulphides in sulphide lead-zinc-iron ores by means of froth flotation comprising the steps of selectively floating lead sulphide leaving a lead tails containing the bulk of the zinc and iron sulphides, and selectively floating zinc sulphide by subjecting said lead tails to froth flotation the improvement which comprises effecting said froth flotation of said lead tails in the presence of 2-mercapto-4,4,6-trimethyl-3,4-dihydropyrimidine. 35

9. In a process for recovering zinc sulfide by froth flotation the step of preparing a mineral

pulp containing the zinc sulfide, incorporating therein as a collector for said zinc sulfide a 2-mercapto - 4 - methyl-4,6-dialkyl-3-4-dihydropyrimidine in which the alkyls are the same radicals selected from the class consisting of methyl and ethyl radicals and subjecting the pulp to froth flotation.

10. In a process for recovering zinc sulfide by froth flotation the step of preparing a mineral pulp containing the zinc sulfide, incorporating therein as a collector for said zinc sulfide a 2-mercapto - 4,4,6 - trimethyl - 3,4-dihydropyrimidine and subjecting the pulp to froth flotation.

WILLIAM H. HILL.

#### REFERENCES CITED

The following references are of record in the file of this patent:

#### UNITED STATES PATENTS

| Number    | Name           | Date          |
|-----------|----------------|---------------|
| 1,364,307 | Perkins -----  | Jan. 4, 1921  |
| 1,364,308 | Perkins -----  | Jan. 4, 1921  |
| 1,364,859 | Perkins -----  | Jan. 4, 1921  |
| 1,610,217 | Elley -----    | Dec. 7, 1926  |
| 1,652,060 | Smith -----    | Dec. 6, 1927  |
| 1,801,317 | Moses -----    | Apr. 21, 1931 |
| 1,801,318 | Moses -----    | Apr. 21, 1931 |
| 1,801,319 | Moses -----    | Apr. 21, 1931 |
| 1,801,320 | Moses -----    | Apr. 21, 1931 |
| 1,933,962 | Bogemann ----- | Nov. 7, 1933  |
| 2,126,269 | Messer -----   | Aug. 9, 1938  |
| 2,234,848 | Horst -----    | Mar. 11, 1941 |

#### OTHER REFERENCES

Giudice, Collection in Flotation, Engineering and Mining Journal, May 1934, pages 213, to 215.

Guitzeit Technical Paper No. 2077 in Mining Technology, 1946, pages 2, 3, 15.

Perry, Chemical Engineer's Handbook, second edition, © 1941, by McGraw-Hill Book Co., page 1736.

Geiser: Technical paper 401, American Inst. of Mining and Met. Engineering, pages 1 to 9.